

## UNITED STATES PATENT OFFICE

2,370,959

METHOD OF HEAT TREATMENT FOR  
WIRE DRAWING

Artemas F. Holden, Northford, Conn.

No Drawing. Application March 4, 1942,  
Serial No. 433,291

1 Claim. (Cl. 148—7)

The present invention relates broadly to metallurgy and more especially to a salt bath method for treating metals, especially ferrous metals, during wire drawing operations.

In order that the present invention may be more clearly understood, a description of the present method of treating metals, particularly steel, during wire drawing operations, is presented. In the common practice of wire drawing, the work is unwound from coils on reels and is heated to a temperature between 1500° F. and 1700° F. either in lead baths or open air furnaces as the first step, and then as a second step, the metal passes through air to a lower temperature stage usually referred to as a quenching stage in which the temperature is lowered to between 900° F. and 1100° F. and this operation may also be carried out either in a lead bath or in an air furnace. The steel is then submitted to a third quenching operation, which may be by the use of a water spray, but more usually merely by permitting it to cool in air. The temperature of the metal on leaving this third stage, is normal atmospheric temperature or slightly higher. After passing the third stage, the steel is recoiled on mechanical reels. The coils are removed from the reels and are submersed in an acid pickling bath where they remain until the deep oxide or scale which is formed on the metal is removed. The fifth step is to submerge the coils in a washing bath to remove the acid pickle and the sixth step is to submerge the coil in a boiling water lime solution which is in the nature of a thick creamy liquid. The coils are taken, in the seventh step, from the lime bath to a baking oven which is heated to a sufficient temperature, usually about 350° F., to quickly evaporate the water and to leave a lime deposit on the wire. The coil is again set on a suitable reel from which the material on the coil is unwound as it is pulled through a drawing die. Preceding the drawing die is a container for suitable grease through which the wire or rod, depending on the diameter of the work, is drawn. The lime coating on the work neutralizes the acid pickling bath and the lime residue deposited on the work picks up and carries with it the grease used for lubrication during the drawing operation.

The drawing of the metal through the drawing dies, where there is a substantial reduction in size, changes the characteristics of the metal and heat treatment is required prior to the next succeeding drawing operation. Therefore, the usual practice is to repeat all the foregoing operations prior to each drawing operation, with the excep-

tion of preceding the final and last draw. The final and last draw is a finishing operation wherein the reduction in size is very slight and the heat treatment step is, therefore, usually omitted prior to the final and last draw; and usually there is no heat treatment after the final and last drawing operation.

The present method comprises the use of salt baths which have related characteristics in such manner that the material of the preceding bath which remains on the work is not substantially removed by the succeeding bath. Thus, the hot stock is completely coated after the stock or work leaves the high temperature bath and until it is cooled sufficiently to prevent uncontrolled oxidation due to oxygen picked up from the air.

In the present invention, the wire stock, after leaving the reel, is first heated in a bath, operating at a temperature between 1500° F. and 1700° F. comprising alkali metal chlorides and an alkali metal fluoride. This bath may comprise 25% to 45% potassium chloride, 35% to 55% sodium chloride, and 1% to 5% sodium fluoride; the preferred specific amounts being 43% potassium chloride, 55% sodium chloride, and 2% sodium fluoride. The work then proceeds to the second bath which comprises an alkali metal hydroxide, an alkali metal chloride, an alkali metal carbonate, an alkali metal fluoride, and an alkali metal cyanide, the preferred range of proportions being 25% to 50% sodium hydroxide, 5% to 20% sodium chloride, 15% to 35% sodium carbonate, 10% to 17% sodium fluoride and 7% to 20% sodium cyanide; the preferred specific proportions being 40% sodium hydroxide or potassium hydroxide, 10% sodium chloride, 25% sodium carbonate, 13% sodium fluoride, and 11% sodium cyanide.

The second bath is intended to operate at temperatures between 900° F. and 1100° F. and the work in passing through the second bath does not lose in any substantial amount the material of the first bath. This is partly due to the fact that the first bath melts at a higher temperature than the second bath and also due to the chemical constituents of the two baths. The advantage of carrying the first bath through the second bath is to prevent contamination of the second bath by the first bath, and to keep the work completely covered by salts while the metal is hot.

In the third step, the work is carried through a water bath. Since the ingredients of the first two baths are soluble in water, the water bath becomes charged with the materials of the first

55 and second bath and the cooled stock leaves the

water bath wetted with a water solution containing the salts of the two preceding baths. The water should contain not less than 4 oz. to 6 oz. of the salts per gallon of water, and in starting it may be desirable to dissolve some of the salts in the water. Therefore, as the water evaporates, a small proportion of these salts remains upon the stock when it is reeled into coils after passing through the baths specified. These treated coils of wire are now ready for a drawing operation without the pickling, liming or baking steps previously referred to in the old well-known ordinary methods. The chemicals remaining on the wire, in accordance with the present invention, are sufficient to act as carriers for the lubricant needed in the drawing operation, and, therefore, the material is ready for a draw as soon as it is passed through the three steps specified as comprising the present invention. These three steps are repeated on all the intermediate draws prior to the last and final draw which brings the stock down to the finished sized wire desired.

The steps of the present invention previously specified may be slightly modified by using a clear water wash which is flowed or sprayed at a sufficient rate to completely wash all of the salts from the wire after the stock has passed the second bath. The material may then be subjected to a very hot lime bath so that when the stock leaves the lime bath it may be of sufficient temperature to dry the lime on the stock without baking, or if desired, the baking step may be included. In any event, the pickling of the wire is omitted according to the present invention. When wire stock is submitted to the steps specified comprising the present invention, the stock is without oxide and is clean, bright metal.

As a further variation of possible treatment, in accordance with the present invention, after the stock has passed the second salt bath and has been washed clean of the first two baths specified, the stock may be passed through a bath comprising a nitrate bath which may be made up of 50% sodium nitrate and 50% potassium nitrate, or 50% sodium hydroxide and 50% sodium nitrate heated to a temperature sufficient to produce a definitely controlled, extremely thin oxide film on the wire. This film is so thin that it cannot be measured by ordinary methods. The potassium nitrate-sodium nitrate bath should be run at a temperature of from 600° F. to 900° F. and would produce a thin film of oxide of a blue-black color, while the sodium hydroxide-sodium nitrate bath, when heated from 900° F. to 1000° F. produces a black oxide. The nitrate bath works very quickly so, therefore, the stock may be passed quickly through this bath in order to obtain the particular controlled oxide desired. This oxide acts as a carrier for a lubricant during the succeeding drawing operation but the metal, after leaving the drawing die, is substantially clear and clean and the oxide has disappeared.

A further slight modification comprises substituting the old lead bath for the first salt bath, and running the lead bath at temperatures of

1500° F. to 1700° F. Where the lead bath is used, there will be a very slight oxidation of the work before the work reaches the second bath which is the salt bath. Since this second bath is a reducing bath, the work leaves the second bath bright and clear of oxide.

The bath No. 1 comprising potassium chloride, sodium chloride, and sodium fluoride may be varied by substituting either potassium carbonate or sodium carbonate for the potassium chloride or the sodium chloride or both. The barium fluoride or calcium fluoride may be substituted for the sodium fluoride. These substances, however, comprise chemical compounds which may tend to contaminate the second bath, and, therefore, are not as desirable as the preferred forms given above.

The second bath may be varied by omitting the alkali metal chloride, and the alkali metal carbonate. When this is done, the bath is more liable to fume and, therefore, the preferred formula is better for the purpose intended.

The melting point of the second bath may be lowered by the addition of potassium hydroxide but the preferred temperatures above specified are those which are most desirable.

One of the prime objects of the present invention is that the stock, after having been heated to the higher temperature, remains coated by chemicals which are inert to the stock until the temperature has been reduced to normal or room temperature, thereby avoiding a heavy film of oxides on the stock which may result in scale which is undesirable.

35 I claim:

The method of preparing ferrous wire for drawing which comprises progressively passing said wire through a salt bath having a temperature of between 1500° and 1700° F. and a composition 40 consisting essentially of from 25% to 45% potassium chloride, 35% to 55% sodium chloride and 1% to 5% sodium fluoride which leaves a ferrous-oxidation inhibiting drag-out coating of said salts thereon, thence progressively passing 45 said thus coated wire through a salt bath having a temperature of between 900° and 1100° F. and a composition consisting essentially of from 25% to 50% sodium hydroxide, 5% to 20% sodium chloride, 15% to 35% sodium carbonate, 10% to 50 17% sodium fluoride and 7% to 20% sodium cyanide which leaves a ferrous-oxidation inhibiting drag-out coating of the salts from both baths upon the wire, thence passing the two-bath coated wire through an aqueous saline bath containing dissolved salts of said baths in a concentration of not less than 4 ounces per gallon to provide upon said wire a thin aqueous coating of the salts of said first two baths, drying said aqueous coating in situ upon said wire to provide a very thin oxidation-protective lubricant-wettable adherent salt coating thereon, and finally applying to said very thin salt coating of said wire a die lubricant which wets and is retained by said salt coating.

ARTEMAS F. HOLDEN.